# EUROPEAN PATENT SPECIFICATION

(11) **EP 3 425 074 B1**
(45) Date of publication and mention of the grant of the patent: **13.01.2021**
(21) Application number: 17181963.4
(22) Date of filing: 18.07.2017
(51) Int. Cl.: C22C 21/12

(54) **SUBSTANTIALLY PB-FREE ALUMINUM ALLOY COMPOSITION**
IM WESENTLICHEN BLEIFREIE ALUMINIUMLEGIERUNG
COMPOSITION D'ALLIAGE D'ALUMINIUM SENSIBLEMENT EXEMPT DE PB

(30) Priority: 03.07.2017 US 201715640722
(43) Date of publication of application: 09.01.2019
(73) Proprietor: Kaiser Aluminum Fabricated Products, LLC, Foothill Ranch, CA 92610-2831 (US)
(72) Inventor: ILDENIZ, Emre, Jackson, TN 38305 (US); MATUSKA, Robert A., Heath, OH 43056 (US); SHOEMAKER, Dave J., Heath, OH 43056 (US)
(74) Representative: FRKelly

(56) References cited:
- CN-A- 101 294 249
- JP-A- 2001 240 931
- JP-A- 2004 002 947
- JP-A- 2006 077 298
- US-A- 5 803 994
- SPIEKERMANN P: "LEGIERUNGEN - EIN BESONDERES PATENTRECHTLICHES PROBLEM? - LEGIERUNGSPRUEFUNG IM EUROPAEISCHEN PATENTAMT -", MITTEILUNGEN DER DEUTSCHEN PATENTANWAELTE, HEYMANN, KOLN, DE, 1 January 1993 (1993-01-01), pages 178-190, XP000961882, ISSN: 0026-6884

## Description

### BACKGROUND OF THE INVENTION

### 1. Field of the Invention

The present invention relates to a substantially Pb-free aluminum alloy composition, and method for making said alloy composition, while achieving the machinability characteristics of their Pb-containing counterparts.

### 2. Description of Related Art

Historically Pb-containing aluminum alloys such as 2011 and 6262 (registered with the Aluminum Association in 1954 and 1960, respectively) have been used for demanding machinability applications. These applications require an alloy that can be machined at high material removal rates while maintaining good machined surface finishes and producing machine chips that are small and easily removed from the work area to prevent jamming the machine tools. Aluminum alloys containing Pb met this need by providing intermetallic phases that acted as chip breakers in the material which enabled faster material removal rates, small machine chips and good machined surfaces. While Pb does provide an effective solution, it is a heavy metal and considered a hazardous material.

In an effort to reduce the adverse health effects and environmental risk these alloys may pose, alternative Pb-free aluminum alloys capable of similar machinability performance are desired. There have been several attempts at developing free machining / Pb free alloys over the years including alloys 2012, 2111, 6020 and 6040. These alloys utilized Bi and / or Sn as a substitute for Pb. While many of these alloys were successful from a machining chip size and machined surface finish perspective, many producers of thin wall, complex parts found they could not achieve the material removal rates that were attained with Pb bearing incumbent alloys because the parts had a tendency to crack. Many of these alloys were thus taken off the market or customers were cautioned to limit material removal rates for some applications. This is problematic, considering many of the applications for the Pb bearing aluminum alloys are sold through distribution channels so the end machining application was unknown to the material producer.

In an effort to avoid potential failures as a result of this crack tendency, the Pb-free alternative alloys that are still available are often restricted in their availability and often have limits placed on the machining parameters that do not achieve the same levels of performance as the Pb-containing alternatives. As a result there is still a market need for a product that meets the machinability characteristics of the Pb-containing alloys, while also meeting the strength requirements. Typically, for example, Pb-containing alloy 2011-T3 has a minimum yield strength of 38 KSI / 262 MPa.

A related alloy employing similar alloying elements is disclosed in CN 101 294 249 A. However, this document works with preferred ranges for Bi: 0.45-0.70 and Sn: 0.2-0.3, which lie above the Bi/Sn ratio1.32/1 specified in claims 1 and 5.

### BRIEF SUMMARY OF THE INVENTION

The substantially Pb-free aluminum alloy composition of the present invention provides a free machining product that achieves the same or superior machining performance in terms of high material removal rates, machining chip size and machined surface finish as their incumbent Pb-containing predecessors.

The substantially Pb-free aluminum alloy composition of the present invention is not susceptible to cracking in thin wall, complex machining under severe material removal conditions. This is a critical distinction that has not been achieved in other inventions attempting to solve the afore-mentioned technical problem. Materials that are susceptible to such cracking conditions render the machining performance irrelevant either by requiring substantially lower material removal rates or disqualifying the material altogether to ensure the integrity of the final part.

The substantially Pb-free aluminum alloy composition of the present invention substantially meets or exceeds the material property requirements of the current free machining materials. Specifically, in a preferred embodiment, the substantially Pb-free aluminum alloy composition meets the minimum material properties for AA2011-T3 including Ultimate Tensile Strength ≥ 45.0 KSI / 311 MPa, Yield Strength ≥ 38.0 KSI / 262 MPa, and % Elongation minimum ≥ 10%.

The substantially Pb-free aluminum alloy composition consists of the following components (in weight percent): Si < 0.40; Fe < 0.70; Cu 5.0 - 6.0; Zn < 0.30; Bi 0.20 - 0.80; Sn 0.10 - 0.50 wherein Si, Fe, Cu, Zn, Bi, and Sn are the only components intentionally added to the alloy composition such that any other material exist only as incidental impurities, with the remainder being aluminum and the incidental impuritiesThe substantially Pb-free aluminum alloy composition maintains a Bi/Sn ratio of less than 1.32/1 (in terms of weight percent; 1.32/1 being the eutectic ratio for Bi-Sn). In addition to this, producing the material in a T8 temper provides specific advantages for machining applications that are sensitive to machining cracks because of their high material removal rates and thin wall geometries. Conversely, specific machining applications that are not sensitive to machining cracks because of more robust part geometries, but which would benefit from even higher material removal rates can be produced in a T6 temper.

### BRIEF DESCRIPTION OF THE DRAWINGS

The features and advantages of the present invention will become apparent from the following detailed description of a preferred embodiment thereof, taken in conjunction with the accompanying drawings, in which:
FIG. 1 is a schematic showing the operational process sequence for the substantially Pb-free aluminum alloy composition produced in the various examples in accordance with the present invention;
FIG. 2 is a conceptual drawing of the representative part used for evaluating machinability from a chip size perspective of a substantially Pb-free aluminum alloy composition in accordance with the present invention;
FIG. 3 is a graph showing machinability for alloy / temper combinations evaluated in Example 1, as measured in chips / gram;
FIG. 4 is a conceptual drawing of the machining crack susceptibility test part;
FIG. 5 shows pictures of observations made from the Machine Crack Susceptibility Test showing the four classifications used;
FIG. 6 is a graph showing Machining Crack Susceptibility Test results for Example 1 as measured in % with no tears or blowouts;
FIG. 7 is a graph showing Machinability results for Example 2 as measured by chips / gram;
FIG. 8 is a graph showing Machining Crack Susceptibility Test results for Example 2 as measured in % with no wrinkles, tears or blowouts;
FIG. 9 is a graph showing machinability results for Example 3 as measured by chips / gram;
FIG. 10 is a graph showing machinability results for Example 3 as measured by chips / gram for 2.000" diameter rod; and
FIG. 11 is a Bi - Sn Phase Diagram.

### DETAILED DESCRIPTION OF THE INVENTION

The substantially Pb-free aluminum alloy composition consists of the following components (in weight percent): Si < 0.40; Fe < 0.70; Cu 5.0 - 6.0; Zn < 0.30; Bi 0.20 - 0.80; Sn 0.10 - 0.50 with the remainder being aluminum and incidental impurities. Si, Fe, Cu, Zn, Bi, and Sn are the only components intentionally added to the alloy composition such that any other material exists only as the incidental impurities. Said incidental impurities are present in a total amount of less than 1 wt.%, or less than 0.5 wt.%, or less than 0.1 wt.%, or less than 0.05 wt.%. The substantially Pb-free aluminum alloy composition maintains a Bi/Sn ratio of less than 1.32/1 (in terms of weight percent; 1.32 being the eutectic ratio for Bi-Sn).

Preferably, the substantially Pb-free aluminum alloy composition of the present invention substantially meets or exceeds the material property requirements of the current free machining materials. Specifically, in a preferred embodiment, the substantially Pb-free aluminum alloy composition meets the minimum material properties for AA2011-T3 including Ultimate Tensile Strength ≥ 45.0 KSI / 311 MPa, Yield Strength ≥ 38.0 KSI / 262 MPa, and % Elongation minimum ≥ 10%.

Generally, the phrase "substantially Pb-free" is defined as having no intentional additions of Pb to the aluminum alloy composition as it is being produced. Preferably, any Pb that may be contained in the aluminum alloy composition is the result of tramp contamination. In a preferred embodiment, the aluminum alloy composition of the present invention contains <0.05 wt.% Pb. In another embodiment, the aluminum alloy composition of the present invention contains <0.01 wt.% Pb. In another preferred embodiment, the aluminum alloy composition of the present invention contains <0.005 wt.% Pb. In another preferred embodiment, the aluminum alloy composition of the present invention contains ≤0.003 wt.% Pb.

It is understood that the ranges identified above for the substantially Pb-free aluminum alloy composition include the upper or lower limits for the element selected and every numerical range and fraction provided within the range may be considered an upper or lower limit. For example, it is understood that within the range of Si < 0.40, the upper or lower limit for Si may be selected from 0.30, 0.25, 0.20, 0.15, and 0.10 wt.%. In one embodiment, the amount of Si ranges from < 0.20 wt.%. In another embodiment, the amount of Si ranges from <0.16 wt.%. In another embodiment, the amount of Si ranges from 0.10-0.16 wt.%. For example, it is also understood that, within the range of Fe < 0.70, the upper or lower limit for Fe may be selected from 0.60, 0.50, 0.40, 0.30, 0.20, and 0.10 wt.%. In one embodiment, the amount of Fe ranges from 0.30-0.50 wt.%. In another embodiment, the amount of Fe ranges from 0.33-0.44 wt.%. For example, it is also understood that within the range of Cu 5.0 - 6.0, the upper or lower limit for Cu may be selected from 5.1, 5.2, 5.3, 5.4, 5.5, 5.6, 5.7, 5.8, and 5.9. In one embodiment, the amount of Cu ranges from 5.1-5.8 wt.%. In another embodiment, the amount of Cu ranges from 5.13-5.63 wt.%. For example, it is also understood that, with the range of Zn < 0.30, the upper or lower limit for Zn may be selected from 0.20, 0.10, 0.05, 0.01, and 0.005 wt.% In one embodiment, the amount of Zn ranges from 0.002-0.05. In another embodiment, the amount of Zn ranges from 0.002-0.044. For example, it is also understood that within the range of Bi 0.20 - 0.80, the upper or lower limit for Bi may be selected from 0.30, 0.40, 0.50, 0.60, and 0.70. In one embodiment, the amount of Bi ranges from 0.40-0.80. In another embodiment, the amount of Bi ranges from 0.20-0.40. For example, it is also understood that within the range of Sn 0.10 - 0.50, the upper or lower limit for Sn may be selected from 0.20, 0.30, and 0.40. In one embodiment, the amount of Sn ranges from 0.20-0.50. Additionally, for example, it is also understood that within the range of Bi/Sn ratio of less than 1.32/1, the upper or lower limit for Bi/Sn ratio may be selected from 1.30/1, 1.25/1, 1.20/1, 1.15/1,1.10/1, 1.05/1, 1.00/1, and 0.80/1. In one embodiment, the Bi/Sn ration may be between 1.32/1-0.80/1. It is further understood that any and all permutations of the ranges identified above are included within the scope of the present invention. For example, the substantially Pb-free aluminum alloy composition may consist of the following components (in weight percent): Si < 0.16; Fe < 0.50; Cu 5.1-5.8; Zn < 0.05; Bi 0.20 - 0.50; Sn 0.20 - 0.50 with the remainder being aluminum and incidental impurities, while maintaining a Bi/Sn ratio of less than 1.32/1 (in terms of weight percent; 1.32/1 being the eutectic ratio for Bi-Sn) or a Bi/Sn ratio from 1.32/1 to 0.80/1, having incidental impurities present in a total amount of less than 1 wt.%, or less than 0.5 wt.%, or less than 0.1 wt.%, or less than 0.05 wt.%.

In addition to this, producing the material in a T8 temper provides specific advantages for machining applications that are sensitive to machining cracks because of their high material removal rates and thin wall geometries. As such, a free machining, machining crack insensitive aluminum alloy may be produced. The aluminum alloy product has been homogenized to improve the recrystallization for improved grain size control. The alloy has a Bi/Sn ratio (in weight percent) of less than 1.32/1. In a preferred embodiment, the alloy has a Bi/Sn ratio (in weight percent) ranging from 1.32/1 to 0.8/1. In yet another preferred embodiment, the alloy has a Bi/Sn ratio (in weight percent) ranging from 1.20/1 to 1/1.

Conversely, specific machining applications that are not sensitive to machining cracks because of more robust part geometries, but which would benefit from even higher material removal rates can be produced in a T6 temper. As such, a superior free machining aluminum alloy material for applications that do not require machine crack insensitive properties may be produced. The aluminum alloy product has been homogenized to improve the recrystallization for improved grain size control. The alloy has a Bi/Sn ratio (in weight percent) is less than 1.32/1. In a preferred embodiment, the alloy has a Bi/Sn ratio (in weight percent) ranging from 1.32/1 to 0.8/1. In yet another preferred embodiment, the alloy has a Bi/Sn ratio (in weight percent) ranging from 1.20/1 to 1/1.

It is important to note that the preferred process in accordance with the present application does not include any naturally aging beyond that which is inherent in the described processes disclosed herein. Specifically, the present invention does not include any T3 or T4 naturally aging of the alloy composition.

Preferred processes for making the alloy composition of the present invention are similar to the processes described in US Patent 5,776,269 and US Patent 5,916,385. The alloy may initially be cast into ingots and the ingots homogenized at a temperature ranging from about 482-571°C (900° to 1170° F) for at least 1 hour but generally not more than 24 hours, optionally followed either by fan or air cooling. In one embodiment, the ingot is soaked at about 548.8 ° C (1020° F) for about 4 hours and then cooled to room temperature. Next, in one embodiment, the ingots are cut into shorter billets, heated to a temperature ranging from about 260° to 382.2° C (500° to 720° F) and then extruded into a desired shape. However, it should be understood that one of ordinary skill in the art may select different times and temperatures and still remain within the scope of the present invention.

In one embodiment, the extruded alloy shapes are then thermomechanically treated to obtain the desired mechanical and physical properties. For example, to obtain the mechanical and physical properties of a T8 temper, solution heat treatment is conducted at a temperature ranging from about 498.9° to 554.4 ° C (930° to 1030° F), preferably at about 537.8° C (1000° F), for a time period ranging from about 0.5 to 2 hours, water quenched to room temperature, cold worked, and artificial aged at a temperature ranging from about 121.1° to 204.4° C (250° to 400° F) for about 2 to 12 hours. However, it should be understood that one of ordinary skill in the art may select different times, quenching conditions, and temperatures and still remain within the scope of the present invention.

In one embodiment, to obtain the properties of a T6 of T6511 temper, prior to extrusion, the billets are homogenized at a temperature ranging from about 510° to 565.6° C (950° to 1050° F) and then extruded to a near desired size. The rod or bar is then straightened using any known straightening operation such as stress relieved stretching of about 1 to 3 %. To further improve its physical and mechanical properties, the alloy is heat treated by precipitation artificial age hardening. Generally, this may be accomplished at a temperature ranging from about 121.1° to 204.4° F (250° to 400° F) for a time period from about 2 to 12 hours. However, it should be understood that one of ordinary skill in the art may select different times, quenching conditions, and temperatures and still remain within the scope of the present invention.

The following examples illustrate various aspects of the invention and are not intended to limit the scope of the invention.

### Example 1:

Billets were produced in 254 mm (10 inch) diameter with the target compositions found in Table 1. These billets were extruded and processed into T3, T4, T6 and T8 tempers using the process parameters shown in FIG.1 to produce 25.4 mm (1.000 inch) diameter rod. Casting of the billets was done using conventional direct chill casting techniques. The 6040 alloy variants were produced in both press quenched (T6511 temper) and separate solution heat treatment (T651 temper) processes. Homogenization, extrusion, solution heat treatment, quenching, drawing and artificial aging operations were all completed using typical industry practices. Samples from this material were evaluated for tensile properties and machinability. The tensile property results are shown in Table 2. The mechanical property limits for 2011-T3 were used as a minimum acceptable criteria. These results show that all but BISN-31-T451 materials pass the aluminum association minimum properties for 2011-T3 (Yield Strength 262 MPa (38.0 KSI); Ultimate Strength 311 MPa (45.0 KSI); 10% Elongation).

**Table 1: Compositions for Example 1 (weight percent)**

| Alloy | Cast | Si | Fe | Cu | Mn | Mg | Zn | Cr | Pb | Bi | Sn | Ti | Zr | B | Ni |
|---|---|---|---|---|---|---|---|---|---|---|---|---|---|---|---|
| BISN-01 | 0969 | 0.11 | 0.36 | 5.22 | 0.00 | 0.00 | 0.044 | 0.020 | 0.001 | 0.40 | 0.35 | 0.020 | 0.003 | 0.001 | 0.00 |
| BISN-03 | 0971 | 0.11 | 0.38 | 5.32 | 0.00 | 0.00 | 0.003 | 0.000 | 0.002 | 0.49 | 0.27 | 0.025 | 0.002 | 0.001 | 0.00 |
| BISN-31 | 0973 | 0.12 | 0.42 | 5.40 | 0.00 | 0.00 | 0.004 | 0.000 | 0.002 | 0.63 | 0.49 | 0.019 | 0.002 | 0.001 | 0.00 |
| BISN-31 | 0975 | 0.12 | 0.39 | 5.47 | 0.00 | 0.00 | 0.003 | 0.000 | 0.002 | 0.60 | 0.42 | 0.022 | 0.002 | 0.001 | 0.00 |
| BISN-31 | 0977 | 0.11 | 0.40 | 5.40 | 0.00 | 0.00 | 0.003 | 0.000 | 0.002 | 0.60 | 0.42 | 0.021 | 0.002 | 0.001 | 0.00 |
| BISN-04 | 0978 | 0.12 | 0.44 | 5.63 | 0.00 | 0.00 | 0.003 | 0.000 | 0.001 | 0.85 | 0.50 | 0.029 | 0.002 | 0.001 | 0.00 |
| BISN-06 | 0979 | 0.13 | 0.40 | 5.16 | 0.00 | 0.00 | 0.002 | 0.000 | 0.001 | 0.57 | 0.45 | 0.024 | 0.002 | 0.000 | 0.00 |
| 2111-06 | 0981 | 0.12 | 0.35 | 5.37 | 0.00 | 0.00 | 0.003 | 0.000 | 0.001 | 0.64 | 0.20 | 0.025 | 0.002 | 0.000 | 0.00 |
| 2111-31 | 0983 | 0.12 | 0.33 | 5.13 | 0.00 | 0.00 | 0.003 | 0.000 | 0.001 | 0.56 | 0.20 | 0.023 | 0.002 | 0.001 | 0.00 |
| BISN-02 | 0985 | 0.13 | 0.39 | 5.34 | 0.00 | 0.00 | 0.009 | 0.002 | 0.001 | 0.67 | 0.60 | 0.015 | 0.002 | 0.001 | 0.00 |
| SNBI-CU | 0986 | 0.11 | 0.36 | 4.36 | 0.00 | 0.00 | 0.003 | 0.000 | 0.001 | 0.59 | 0.41 | 0.023 | 0.002 | 0.002 | 0.00 |
| SNBI-NI | 0989 | 0.13 | 0.40 | 5.24 | 0.00 | 0.00 | 0.003 | 0.000 | 0.005 | 0.58 | 0.42 | 0.013 | 0.002 | 0.001 | 1.51 |
| TEN6040 | 40-1 | 0.60 | 0.44 | 0.56 | 0.11 | 0.93 | 0.090 | 0.055 | 0.006 | 0.17 | 0.89 | 0.020 | 0.002 | 0.000 | 0.00 |
| LAX6040 | 0445 | 0.72 | 0.29 | 0.43 | 0.07 | 0.95 | 0.170 | 0.078 | 0.025 | 0.29 | 0.85 | 0.036 | 0.000 | 0.000 | 0.00 |

The alloys identified as BISN-01, BISN-31 (casts 0973 and 0975 and 0977), BISN-06, 2111-06, 2111-31 and SNBI-NI form part of the present invention.

**Table 2: Mechanical Properties of Material Evaluated in Example 1**

| Lot ID | Cast # | Alloy | Temper | Yield MPa (KSI) | Ultimate MPa (KSI) | % Elongation |
|---|---|---|---|---|---|---|
| 299 | 969 | BISN-01 | T3 | 317 (45.9) | 361 (52.3) | 17.2 |
| 300 | 985 | BISN-02 | T3 | 318 (46.1) | 363 (52.5) | 15.0 |
| 301 | 971 | BISN-03 | T3 | 313 (45.3) | 355 (51.5) | 16.5 |
| 302 | 978 | BISN-04 | T3 | 319 (46.3) | 363 (52.6) | 15.3 |
| 303 | 975 | BISN-31 | T3 | 317 (46.0) | 362 (52.4) | 16.5 |
| 304 | 973 | BISN-31 | T451 | 169 (24.5) | 303 (43.9) | 33.8 |
| 306 | 979 | BISN-06 | T3 | 307 (44.5) | 346 (50.2) | 16.8 |
| 307 | 983 | 2111-31 | T3 | 302 (43.8) | 342 (49.6) | 17.3 |
| 308 | 981 | 2111-06 | T3 | 314 (45.5) | 355 (51.4) | 15.8 |
| 310 | 989 | BISN-NI | T3 | 268 (38.9) | 296 (42.9) | 13.0 |
| 311 | 986 | BISN-CU | T3 | 278 (40.3) | 311 (45.1) | 16.5 |
| 305 | 977 | BISN-31 | T8 | 290 (42.1) | 386 (55.9) | 15.2 |
| 233 | 001 | 2011 | T3 | 323 (46.8) | 356 (51.6) | 15.5 |
| 312 | 822 | 6040 | T651 | 308 (44.6) | 340 (49.3) | 18.5 |
| 000 | 000 | 6040 | T6511 | 361 (52.3) | 384 (55.6) | 13.0 |

The alloys identified as BISN-01, BISN-31 (casts 0973 and 0975 and 0977), BISN-06, 2111-06, 2111-31 and SNBI-NI form part of the present invention.

Machinability testing was conducted by producing a representative part that utilizes several machining operations. This part is depicted conceptually in FIG. 2. Material removal rates were kept constant between materials by keeping the cutting speed and feed rate constant for all machining operations. The chip size is evaluated by determining the number of clean, dry chips per gram. The results from this evaluation are shown in FIG.3 and are compared with current Pb-containing free machining material, 2011-T3, as a benchmark comparison. This shows that the alloy / temper combinations tested were better or comparable to the incumbent material. Also tested in this matrix were Pb-free 6040 compositions that are currently available in the market. These have historically not performed as well as 2011-T3, and this test validated their inferior performance.

In order to test that the materials were not susceptible to cracking in thin wall, severe machining applications, a severe machining test was developed. This involves drilling out the center of the 25.4 mm (1.000") rod using 24.6 mm (0.969") diameter twist drill, resulting in a 0.38 mm (0.015") wall thickness, as shown in FIG.4. The RPM and feed rate was kept constant at 1500 RPMs and 1.27 mm (0.035") / revolution feed rate. Once this test was completed, the specimens were examined for conditions as depicted in FIG. 5. This test was developed for testing the materials susceptibility to cracking under extreme machining conditions with thin walls, high material removal rates and high torque applied. This test was replicated a minimum of 12 times for each material tested that had acceptable performance from a chip size and material property perspective. The percentage of parts with tears (or cracks) and blowouts was recorded and the results are shown in FIG. 6. The BISN-31 is designated with the different tempers (T3, T4 and T8) in this figure for simplification. This shows that the 2011 (incumbent Pb-containing alloy) consistently passed, as expected, as well as the Pb-free 6040 alloy variants (note these alloy variants did not perform well from a chip size perspective, however). The only experimental alloy that passed was BISN-31-T4, but unfortunately this failed the tensile property requirements.

Analysis of these results indicates that alloy / temper combinations with lower yield to ultimate strength ratios perform better from a machining crack susceptibility perspective. Closer analysis of BISN-01 through BISN-04 compositions indicates that lower Bi+Sn content and lower Bi/Sn ratios are beneficial from a machining crack susceptibility perspective when taking into account the severity of the failures. The Bi/Sn ratio appears to be the stronger influence relative to the composition related performance input variables. This is illustrated in Table 3. Note that the Bi-Sn eutectic composition from a weight percent basis is at a ratio of 1.32 Bi/Sn (as shown in FIG. 11).

**Table 3: Severity of Machining Crack Susceptibility Results for Alloys BISN-01 through BISN-04**

| Alloy | Bi+Sn | Bi/Sn | % Wrinkled | % Torn | % Blowout |
|---|---|---|---|---|---|
| BISN-01 | 0.75 | 1.14 | 17% | 77% | 6% |
| BISN-02 | 1.27 | 1.12 | 21% | 50% | 29% |
| BISN-03 | 0.76 | 1.81 | 7% | 13% | 80% |
| BISN-04 | 1.35 | 1.70 | 20% | 20% | 60% |

BISN-01 forms part of the present invention.

### Example 2:

Billets were cast in 254 mm (10") diameter and processed into 25.4 mm (1") rod using the process depicted in FIG.1 and the compositions listed in Table 4. The % ROA (reduction of area) during the drawing operation was evaluated in this study, particularly in the T3 temper. The effect of homogenization was also evaluated with cast 1110 being homogenized and compared to the unhomogenized cast 1108. The 25.4 mm (1") rod was evaluated for mechanical properties, machinability, and machining crack susceptibility using the same techniques described in Example 1.

**Table 4: Compositions of the present invention and Tempers for Example 2 (weight percent)**

| Alloy | Cast | Bi | Sn | Cu | Mg | Fe | Si | Ni | Mn | Pb | Cr | Bi/Sn | Bi+Sn | Temper | % ROA |
|---|---|---|---|---|---|---|---|---|---|---|---|---|---|---|---|
| BI26 | 1102 | 0.27 | 0.24 | 5.31 | 0.00 | 0.42 | 0.15 | 0.00 | 0.00 | 0.00 | 0.00 | 1.13 | 0.51 | T3 | 20.3 |
| BI26 | 1103 | 0.28 | 0.23 | 5.40 | 0.00 | 0.35 | 0.13 | 0.00 | 0.00 | 0.00 | 0.08 | 1.22 | 0.51 | T3 | 15.8 |
| BI26 | 1104 | 0.27 | 0.24 | 5.35 | 0.00 | 0.36 | 0.14 | 0.00 | 0.00 | 0.00 | 0.00 | 1.13 | 0.51 | T3 | 9.3 |
| BI26 | 1105 | 0.26 | 0.24 | 5.36 | 0.00 | 0.38 | 0.15 | 0.00 | 0.00 | 0.00 | 0.00 | 1.08 | 0.50 | T8 | 15.8 |
| BI26 | 1106 | 0.26 | 0.24 | 5.34 | 0.00 | 0.35 | 0.14 | 0.00 | 0.00 | 0.00 | 0.00 | 1.08 | 0.50 | T651 | 17.4 |
| BI39 | 1111 | 0.39 | 0.36 | 5.37 | 0.00 | 0.41 | 0.14 | 0.00 | 0.00 | 0.00 | 0.00 | 1.08 | 0.75 | T3 | 20.3 |
| BI39 | 1108 | 0.37 | 0.35 | 5.31 | 0.00 | 0.39 | 0.15 | 0.00 | 0.00 | 0.00 | 0.00 | 1.06 | 0.72 | T3 | 15.8 |
| BI39 | 1109 | 0.39 | 0.36 | 5.41 | 0.00 | 0.41 | 0.14 | 0.00 | 0.00 | 0.00 | 0.00 | 1.08 | 0.75 | T3 | 9.3 |
| BI39 | 1112 | 0.40 | 0.36 | 5.28 | 0.00 | 0.33 | 0.14 | 0.00 | 0.00 | 0.00 | 0.00 | 1.11 | 0.76 | T8 | 15.8 |
| BI39 | 1113 | 0.40 | 0.36 | 5.24 | 0.00 | 0.40 | 0.14 | 0.00 | 0.00 | 0.00 | 0.00 | 1.11 | 0.76 | T651 | 17.4 |
| BI39 | 1110 | 0.39 | 0.36 | 5.32 | 0.00 | 0.40 | 0.14 | 0.00 | 0.00 | 0.00 | 0.00 | 1.08 | 0.75 | T3 | 15.8 |
| BI39MG | 1114 | 0.40 | 0.37 | 5.47 | 0.50 | 0.42 | 0.14 | 0.00 | 0.00 | 0.00 | 0.00 | 1.08 | 0.77 | T451 | 17.4 |

The mechanical properties are shown in Table 5. This shows that all of the composition and temper combinations were capable of achieving the minimum 2011-T3 target mechanical properties (Yield Strength 262 MPa (38 KSI); Ultimate Strength 311 MPa (45.0 KSI); 10% Elongation). The addition of Mg was successful in achieving these properties as well in the T4 temper.

**Table 5: Mechanical Properties of Material Evaluated in Example 2**

| Lot ID | Cast # | Alloy | % ROA | Temper | Yield MPa (KSI) | Ultimate MPa (KSI) | % Elongation |
|---|---|---|---|---|---|---|---|
| 338 | 1102 | BI26 | 20.3 | T3 | 313 (45.3) | 348 (50.5) | 15.0 |
| 341 | 1103 | BI26 | 15.8 | T3 | 302 (43.8) | 344 (49.8) | 18.0 |
| 344 | 1104 | BI26 | 9.3 | T3 | 275 (39.8) | 322 (46.6) | 18.0 |
| 345 | 1105 | BI26 | 15.8 | T8 | 270 (39.2) | 371 (53.8) | 15.0 |
| 347 | 1106 | BI26 | 17.4 | T651 | 277 (40.2) | 406 (58.8) | 23.0 |
| 339 | 1111 | BI39 | 20.3 | T3 | 324 (46.9) | 355 (51.4) | 14.0 |
| 342 | 1108 | BI39 | 15.8 | T3 | 302 (43.8) | 343 (49.7) | 18.5 |
| 343 | 1109 | BI39 | 9.3 | T3 | 265 (38.4) | 325 (47.1) | 12.0 |
| 346 | 1112 | BI39 | 15.8 | T8 | 270 (39.2) | 372 (53.9) | 14.0 |
| 348 | 1113 | BI39 | 17.4 | T651 | 275 (39.9) | 397 (57.5) | 22.0 |
| 350 | 1110 | BI39 | 15.8 | T3 | 303 (43.9) | 347 (50.3) | 17.0 |
| 351 | 1114 | BI39 | 17.4 | T451 | 267 (38.7) | 402 (58.2) | 20.0 |

The machinability test, relative to chip size was evaluated with the results depicted in FIG. 7. These results show that higher Bi+Sn compositions (BI39) perform better from a machinability perspective, as measured by chips / gram, and perform as good or better than the incumbent 2011-T3. The lower Bi+Sn compositions (BI26) generally did not perform as well as the incumbent 2011-T3, but were comparable. It also shows that there is very little difference on the machinability as related to percent reduction area for T3 tempers, regardless of Bi+Sn levels. The addition of homogenization did not improve the machinability, but examination of the grain structure revealed significant improvement relative to peripheral coarse grain (recrystallized grain size on outer periphery of the rod). Therefore the use of homogenization, while not necessary for machinability, may be beneficial for some applications requiring improved surface appearance (such as parts requiring anodizing). The T651 temper material, regardless of alloy composition, performed very well, with small chip size. The T8 tempers generally performed better than the T3 counterparts for a given alloy, particularly the BI26 composition.

In terms of the machining crack susceptibility test, these results are shown in FIG.8, in this case, wrinkles on the surface (per FIG.5) were also considered unacceptable. These results show that while composition BI26 performed significantly better than BI39 (confirming that higher Bi+Sn makes the material more susceptible to machining cracks), the temper has a much stronger influence. Note that all of the compositions in this example had less than 1.32 Bi/Sn ratios. The T8 tempers did not crack in this test regardless of composition, while the T6 samples performed very poorly. The T3 tempers all had some failures, with the higher Bi+Sn containing materials having significantly higher failure rates. The BI26-T3 compositions had no failures in terms of tears or blow-outs per FIG.5, thus the Bi+Sn has a significant impact on performance.

These results therefore demonstrate that, by producing the material in a T8 temper, higher Bi+Sn levels can be utilized, thus achieving the superior machinability from a chip size perspective as well.

### Example 3:

Billets were cast in 254 mm (10") diameter and processed into 25.4 mm (1") and 50.8 mm (2") T3 and T8 rod using the process depicted in FIG. 1 and the compositions listed in Table 6. The rods were evaluated for mechanical properties, machinability, and machining crack susceptibility using the same techniques described in Example 1.

**Table 6: Compositions of the present invention and Tempers for Example 3 (weight percent)**

| Alloy | Cast | Si | Fe | Cu | Mn | Mg | Zn | Cr | Pb | Bi | Sn | Ti | Bi+Sn | Bi/Sn |
|---|---|---|---|---|---|---|---|---|---|---|---|---|---|---|
| SN01 | 1172 | 0.16 | 0.45 | 5.76 | 0.03 | 0.00 | 0.00 | 0.00 | 0.002 | 0.25 | 0.21 | 0.009 | 0.46 | 1.21 |
| SN01 | 1173 | 0.14 | 0.36 | 5.32 | 0.03 | 0.02 | 0.00 | 0.00 | 0.000 | 0.24 | 0.20 | 0.010 | 0.44 | 1.20 |
| SN02 | 1175 | 0.15 | 0.39 | 5.55 | 0.03 | 0.00 | 0.01 | 0.00 | 0.002 | 0.35 | 0.21 | 0.013 | 0.56 | 1.65 |
| SN02 | 1176 | 0.15 | 0.36 | 5.25 | 0.03 | 0.02 | 0.00 | 0.06 | 0.002 | 0.34 | 0.19 | 0.010 | 0.53 | 1.83 |
| SN03 | 1178 | 0.10 | 0.38 | 5.77 | 0.03 | 0.02 | 0.00 | 0.01 | 0.000 | 0.26 | 0.33 | 0.005 | 0.59 | 0.80 |
| SN03 | 1182 | 0.16 | 0.39 | 5.37 | 0.03 | 0.01 | 0.00 | 0.01 | 0.003 | 0.24 | 0.30 | 0.009 | 0.55 | 0.81 |
| SN04 | 1180 | 0.15 | 0.36 | 5.35 | 0.03 | 0.02 | 0.00 | 0.00 | 0.002 | 0.35 | 0.35 | 0.006 | 0.70 | 1.00 |
| SN04 | 1184 | 0.14 | 0.37 | 5.25 | 0.04 | 0.02 | 0.00 | 0.00 | 0.002 | 0.35 | 0.31 | 0.011 | 0.66 | 1.15 |

The mechanical properties are shown in Table 7. This shows that all of the composition and temper combinations were capable of achieving the minimum 2011-T3 target mechanical properties (Yield Strength 262 MPa (38 KSI); Ultimate Strength 311 MPa (45.0 KSI); 10% Elongation).

**Table 7: Mechanical Properties of Material Evaluated in Example 3**

| Alloy / Temper | Cast | Lot ID | Diameter mm (inch) | Yield MPa (KSI) | Ultimate MPa (KSI) | % Elongation |
|---|---|---|---|---|---|---|
| SN01-T3 | 1172 | 402 | 25.4 (1.000) | 311 (45.0) | 348 (50.4) | 14.0 |
| SN02-T3 | 1175 | 403 | 25.4 (1.000) | 306 (44.4) | 347 (50.3) | 16.0 |
| SN03-T3 | 1182 | 404 | 25.4 (1.000) | 307 (44.5) | 350 (50.7) | 15.0 |
| SN04-T3 | 1184 | 405 | 25.4 (1.000) | 303 (43.9) | 342 (49.6) | 16.0 |
| SN01-T8 | 1173 | 398 | 50.8 (2.000) | 305 (44.2) | 391 (56.6) | 13.0 |
| SN02-T8 | 1175 | 399 | 50.8 (2.000 | 290 (42.1) | 388 (56.2) | 14.0 |
| SN03-T8 | 1182 | 400 | 50.8 (2.000) | 299 (43.3) | 392 (56.8) | 14.0 |
| SN04-T8 | 1184 | 401 | 50.8 (2.000) | 309 (44.8) | 395 (57.2) | 14.0 |
| SN01-T8 | 1172 | 760 | 25.4 (1.000) | 295 (42.7) | 385 (55.8) | 14.0 |
| SN02-T8 | 1176 | 761 | 25.4 (1.000) | 313 (45.4) | 395 (57.3) | 15.0 |
| SN03-T8 | 1178 | 762 | 25.4 (1.000) | 286 (41.5) | 382 (55.3) | 15.0 |
| SN04-T8 | 1180 | 763 | 25.4 (1.000) | 295 (42.8) | 380 (55.0) | 15.0 |

The machinability test relative to chip size was evaluated with the results depicted in FIG. 9 for the 25.4 mm (1.000") diameter material. The results show that the T8 performed superior to the Pb-containing 2011 material, while the T3 material, which still performed acceptably, was not as good as the Pb-containing 2011 material. The test was replicated with the 50.8 mm (2.000") diameter to ensure the material machined well over a wider range of diameters. While the 50.8 mm (2.000") diameter results were slightly worse than the Pb-containing 2011 incumbent material in this test, it must be noted that from a chips per gram basis, it was better than any of the 25.4 mm (1.000") diameter test results. Thus it can be concluded that the material performs well throughout these diameter ranges.

Machining crack susceptibility testing was also performed on the 25.4 mm (1.000") diameter material considering wrinkles, tears and blow-outs (per FIG. 5) as failures. The results of this testing are shown in Table 8.

**Table 8: Summary of Results for the Machining Crack Susceptibility Testing for 25.4 mm (1.000") Diameter Example 3**

| Alloy | Temper | Cast | Lot ID | Bi/Sn | Percent Passing |
|---|---|---|---|---|---|
| SN01 | T3 | 1172 | 402 | 1.21 | 5% |
| SN02 | T3 | 1176 | 403 | 1.83 | 0% |
| SN03 | T3 | 1178 | 404 | 0.80 | 0% |
| SN04 | T3 | 1180 | 405 | 1.00 | 0% |
| SN01 | T8 | 1172 | 760 | 1.21 | 100% |
| SN02 | T8 | 1176 | 761 | 1.83 | 45% |
| SN03 | T8 | 1178 | 762 | 0.80 | 100% |
| SN04 | T8 | 1180 | 763 | 1.00 | 95% |

These results confirm that for applications with severe material removal rates and part geometries with thin walls that are susceptible to tearing, processing the material in a T8 temper and maintaining Bi/Sn ratios less than 1.32 virtually eliminates this failure mechanism.

Although the present invention has been disclosed in terms of a preferred embodiment, it will be understood that numerous additional modifications and variations could be made thereto without departing from the scope of the invention as defined by the following claims:

## Claims

1. A method for forming an aluminum alloy comprising the steps:
a. casting an alloy billet of an aluminum alloy composition, the composition consisting of the following components (in weight percent of the aluminum alloy composition):
Si 0- 0.40; Fe 0- 0.70; Cu 5.0 - 6.0; Zn 0- 0.30; Bi 0.20 - 0.80;
Sn 0.10 - 0.50; wherein Si, Fe, Cu, Zn, Bi, and Sn are the only components intentionally added to the alloy composition such that any other material exist only as incidental impurities, with the balance being aluminum save for the incidental impurities, said alloy composition having a ratio by weight of Bi/Sn of less than 1.32/1;
b. optionally homogenizing the cast billet;
c. extruding the cast billet to form an extrusion having a profile shape;
d. solution heat treating the extrusion by heating to a soak temperature between 482-571°C (900-1060°F) and quenching from the soak temperature to room temperature;
e. cold working the extrusion after step d) via drawing, stretching or rolling to a minimum of 5% reduction of cross sectional area; and
f. artificial aging the extrusion of step e) to peak hardness using only a T8 or T6 temper to produce said aluminum alloy having an Ultimate Tensile Strength ≥ 311 MPa (45.0 KSI), Yield Strength ≥ 262 MPa (38.0 KSI), and % Elongation minimum ≥ 10%.

2. The method of claim 1 wherein
said step of homogenizing the cast billet occurs at a temperature within the range of 482.2-565.6 °C (900-1050 °F) for a time period of not less than 1 hour; and
said step of solution heat treating the extrusion by heating to a temperature between 482.2-571.1°C (900-1060 °F) occurs for 0.5 to 2 hours.

3. The method of claim 1 or 2, wherein said artificial aging includes a T8 temper.

4. The method of any one of claims 1-3, wherein said aluminum alloy is not subjected to a T3 or T4 temper.

5. A substantially Pb-free aluminum alloy composition consisting of the following components (in weight percent of the aluminum alloy composition):
Si 0 -0.40; Fe 0-0.70; Cu 5.0 - 6.0; Zn 0-0.30; Bi 0.20 - 0.80; Sn 0.10 - 0.50; wherein Si, Fe, Cu, Zn, Bi, and Sn are the only components intentionally added to the alloy composition such that any other material exist only as incidental impurities, with the balance being aluminum save for the incidental impurities;
said alloy composition having a ratio by weight of Bi/Sn of less than 1.32/1; and
said alloy composition manufactured using only artificial aging at a T8 or T6 temper to provide an alloy composition having an Ultimate Tensile Strength ≥ 311 MPa (45.0 KSI), Yield Strength ≥ 262 MPa (38.0 KSI), and % Elongation minimum ≥ 10% and wherein said aluminum alloy composition has <0.05 wt. % Pb.

6. The composition of claim 5 wherein said aluminum alloy composition comprises 0.10-0.16 wt. % Si.

7. The composition of any one of claims 5 to 6 wherein said aluminum alloy composition comprises 0.30-0.50 wt. % Fe.

8. The composition of any one of claims 5 to 7 wherein said aluminum alloy composition comprises 5.1-5.8 wt. % Cu.

9. The composition of any one of claims 5 to 8 wherein said aluminum alloy composition comprises 0.002-0.05 wt. % Zn.

10. The composition of any one of claims 5 to 9 wherein said aluminum alloy composition comprises 0.20-0.40 wt. % Bi.

11. The composition of any one of claims 5 to 10 wherein said aluminum alloy composition comprises 0.20-0.50 wt. % Sn.

12. The composition of claim 5 wherein said aluminum alloy composition consists of the following components (in percent (weight / weight) of the aluminum alloy composition):
Si 0-0.16; Fe 0-0.50; Cu 5.1-5.8; Zn 0- 0.05; Bi 0.20 - 0.40; and Sn 0.20 - 0.50.

13. The composition of any one of claims 5 to 12 wherein said aluminum alloy composition has a ratio by weight of Bi/Sn in the range from 1.32/1 to 0.8/1.

14. The composition of any one of claims 5 to 13 wherein said incidental impurities are present in a total amount of less than 0.5 wt. %.

## Patentansprüche

1. Verfahren für die Bildung einer Aluminiumlegierung, das die folgenden Schritte umfasst:
a. Gießen eines Legierungsknüppels einer
Aluminiumlegierungszusammensetzung, wobei die Zusammensetzung aus den folgenden Komponenten (in Gewichtsprozenten der Aluminiumlegierungszusammensetzung) besteht:
Si 0-0,40; Fe 0-0,70; Cu 5,0-6,0; Zn 0-0,30; Bi 0,20-0,80;
Sn 0,10-0,50; wobei Si, Fe, Cu, Zn, Bi und Sn die einzigen Komponenten sind, die absichtlich zu der Legierungszusammensetzung zugegeben werden, sodass jedwedes andere Material nur als zufällige Verunreinigung vorkommt, wobei der Restbetrag Aluminium ist, ausgenommen die zufälligen Verunreinigungen, wobei die Legierungszusammensetzung ein Gewichtsverhältnis von Bi/Sn von kleiner als 1,32/1 aufweist;
b. optionales Homogenisieren des gegossenen Knüppels;
c. Strangpressen des gegossenen Knüppels, um ein Strangpressteil zu bilden, das eine Profilform aufweist;
d. Lösungsglühen des Strangpressteils durch Erhitzen auf eine Durchwärmtemperatur zwischen 482-571 °C (900-1060 °F) und Abschrecken von der Durchwärmtemperatur auf Raumtemperatur;
e. Kaltbearbeiten des Strangpressteils nach Schritt d) über Ziehen, Strecken oder Walzen auf ein Minimum von 5 % Reduzierung der Querschnittsfläche; und
f. künstliches Altern des Strangpressteils von Schritt e) auf eine höchste Härte unter Verwendung von nur einem T8- oder T6-Zustand, um die Aluminiumlegierung herzustellen, die eine Zugfestigkeit von ≥ 311 MPa (45,0 KSI), Streckgrenze von ≥ 262 MPa (38,0 KSI) und ein %-Dehnungsminimum von ≥ 10 % aufweist.

2. Verfahren nach Anspruch 1, wobei
der Schritt des Homogenisierens des gegossenen Knüppels bei einer Temperatur in dem Bereich von 482,2-565,6 °C (900-1050 °F) für eine Zeitdauer von nicht weniger als 1 Stunde auftritt; und
der Schritt des Lösungsglühens des Strangpressteils durch Erhitzen auf eine Temperatur zwischen 482,2-571,1 °C (900-1060 °F) für 0,5 bis 2 Stunden auftritt.

3. Verfahren nach Anspruch 1 oder 2, wobei das künstliche Altern einen T8-Zustand einschließt.

4. Verfahren nach einem der Ansprüche 1-3, wobei die Aluminiumlegierung nicht einem T3- oder T4-Zustand unterzogen wird.

5. Wesentlich Pb-freie Aluminiumlegierungszusammensetzung, die aus den folgenden Komponenten (in Gewichtsprozenten der Aluminiumlegierungszusammensetzung) besteht:
Si 0-0,40; Fe 0-0,70; Cu 5,0-6,0; Zn 0-0,30; Bi 0,20-0,80; Sn 0,10-0,50; wobei Si, Fe, Cu, Zn, Bi und Sn die einzigen Komponenten sind, die absichtlich zu der Legierungszusammensetzung zugegeben sind, sodass jedwedes andere Material nur als zufällige Verunreinigung vorkommt, wobei der Restbetrag Aluminium ist, ausgenommen die zufälligen Verunreinigungen;
wobei die Legierungszusammensetzung ein Gewichtsverhältnis von Bi/Sn von kleiner als 1,32/1 aufweist; und
wobei die Legierungszusammensetzung unter Verwendung von nur künstlichem Altern bei einem T8- oder T6-Zustand hergestellt wurde, um eine Aluminiumlegierung bereitzustellen, die eine Zugfestigkeit von ≥ 311 MPa (45,0 KSI), Streckgrenze von
≥ 262 MPa (38,0 KSI) und ein %-Dehnungsminimum von ≥ 10 % aufweist, und wobei die Aluminiumlegierungszusammensetzung < 0,05 Gew.-% Pb aufweist.

6. Zusammensetzung nach Anspruch 5, wobei die Aluminiumlegierungszusammensetzung 0,10-0,16 Gew.-% Si umfasst.

7. Zusammensetzung nach einem der Ansprüche 5 bis 6, wobei die Aluminiumlegierungszusammensetzung 0,30-0,50 Gew.-% Fe umfasst.

8. Zusammensetzung nach einem der Ansprüche 5 bis 7, wobei die Aluminiumlegierungszusammensetzung 5,1-5,8 Gew.-% Cu umfasst.

9. Zusammensetzung nach einem der Ansprüche 5 bis 8, wobei die Aluminiumlegierungszusammensetzung 0,002-0,05 Gew.-% Zn umfasst.

10. Zusammensetzung nach einem der Ansprüche 5 bis 9, wobei die Aluminiumlegierungszusammensetzung 0,20-0,40 Gew.-% Bi umfasst.

11. Zusammensetzung nach einem der Ansprüche 5 bis 10, wobei die Aluminiumlegierungszusammensetzung 0,20-0,50 Gew.-% Sn umfasst.

12. Zusammensetzung nach Anspruch 5, wobei die Aluminiumlegierungszusammensetzung aus den folgenden Komponenten (in Prozent (Gewicht/Gewicht) der Aluminiumlegierungszusammensetzung) besteht:
Si 0-0,16; Fe 0-0,50; Cu 5,1-5,8; Zn 0-0,05; Bi 0,20-0,40; und Sn 0,20-0,50.

13. Zusammensetzung nach einem der Ansprüche 5 bis 12, wobei die Aluminiumlegierungszusammensetzung ein Gewichtsverhältnis von Bi/Sn in dem Bereich von 1,32/1 bis 0,8/1 aufweist.

14. Zusammensetzung nach einem der Ansprüche 5 bis 13, wobei die zufälligen Verunreinigungen in einer Gesamtmenge von weniger als 0,5 Gew.-% vorliegen.

## Revendications

1. Méthode de formation d'un alliage d'aluminium, comprenant les étapes :
a. de moulage d'une billette d'alliage d'une composition d'alliage d'aluminium, la composition étant constituée des composants suivants (en pourcentage pondéral de la composition d'alliage d'aluminium) :
Si 0-0,40 ; Fe 0-0,70 ; Cu 5,0-6,0 ; Zn 0-0,30 ; Bi 0,20-0,80 ;
Sn 0,10-0,50 ; où Si, Fe, Cu, Zn, Bi et Sn sont les seuls composants ajoutés de manière intentionnelle à la composition d'alliage de sorte que tout autre matériau n'existe que sous forme d'impuretés accessoires, le reste étant constitué d'aluminium à part les impuretés accessoires, ladite composition d'alliage présentant un rapport pondéral de Bi/Sn inférieur à 1,32/1 ;
b. éventuellement, d'homogénéisation de la billette coulée ;
c. d'extrusion de la billette coulée afin de former une extrusion ayant une forme de profil ;
d. de traitement thermique en solution de l'extrusion, par un chauffage jusqu'à une température de trempage entre 482-571°C (900-1060°F) et de trempe à partir de la température de trempage jusqu'à température ambiante ;
e. de travail à froid de l'extrusion après l'étape d) via étirage, cintrage à plat ou laminage jusqu'à un minimum de 5% de réduction de la superficie en coupe ; et
f. de vieillissement artificiel de l'extrusion de l'étape e) jusqu'à une dureté maximale en n'utilisant qu'une trempe T8 ou T6 afin de produire ledit alliage d'aluminium ayant une limite de résistance à la traction ≥ 311 MPa (45,0 KSI), une limite d'élasticité ≥ 262 MPa (38,0 KSI), et un % d'élongation minimum ≥ 10%.

2. Méthode selon la revendication 1, dans laquelle
ladite étape d'homogénéisation de la billette coulée est effectuée à une température dans la plage de 482,2-565,6°C (900-1050°F) pour une période de temps non inférieure à 1 heure ; et
ladite étape de traitement thermique en solution de l'extrusion, par un chauffage jusqu'à une température entre 482,2-571,1°C (900-1060°F) est effectuée pendant de 0,5 à 2 heures.

3. Méthode selon la revendication 1 ou 2, dans laquelle ledit vieillissement artificiel comporte une trempe T8.

4. Méthode selon l'une quelconque des revendications 1-3, dans laquelle ledit alliage d'aluminium n'est pas soumis à une trempe T3 ou T4.

5. Composition d'alliage d'aluminium sensiblement exempte de Pb, constituée des composants suivants (en pourcentage pondéral de la composition d'alliage d'aluminium) :
Si 0-0,40 ; Fe 0-0,70 ; Cu 5,0-6,0 ; Zn 0-0,30 ; Bi 0,20-0,80 ; Sn 0,10-0,50 ; où Si, Fe, Cu, Zn, Bi et Sn sont les seuls composants ajoutés de manière intentionnelle à la composition d'alliage de sorte que tout autre matériau n'existe que sous forme d'impuretés accessoires, le reste étant constitué d'aluminium à part les impuretés accessoires,
ladite composition d'alliage présentant un rapport pondéral de Bi/Sn inférieur à 1,32/1 ; et
ladite composition d'alliage étant fabriquée en n'utilisant qu'un vieillissement artificiel à une trempe T8 ou T6 afin de produire une composition d'alliage ayant une limite de résistance à la traction ≥ 311 MPa (45,0 KSI), une limite d'élasticité ≥ 262 MPa (38,0 KSI), et un % d'élongation minimum ≥ 10% ; et
ladite composition d'alliage d'aluminium contenant <0,05% en poids de Pb.

6. Composition selon la revendication 5, ladite composition d'alliage d'aluminium contenant 0,10-0,16% en poids de Si.

7. Composition selon l'une quelconque des revendications 5 à 6, ladite composition d'alliage d'aluminium contenant 0,30-0,50% en poids de Fe.

8. Composition selon l'une quelconque des revendications 5 à 7, ladite composition d'alliage d'aluminium contenant 5,1-5,8% en poids de Cu.

9. Composition selon l'une quelconque des revendications 5 à 8, ladite composition d'alliage d'aluminium contenant 0,002-0,05% en poids de Zn.

10. Composition selon l'une quelconque des revendications 5 à 9, ladite composition d'alliage d'aluminium contenant 0,20-0,40% en poids de Bi.

11. Composition selon l'une quelconque des revendications 5 à 10, ladite composition d'alliage d'aluminium contenant 0,20-0,50% en poids de Sn.

12. Composition selon la revendication 5, ladite composition d'alliage d'aluminium étant constituée des composants suivants (en pourcentage pondéral de la composition d'alliage d'aluminium) :
Si 0-0,16 ; Fe 0-0,50 ; Cu 5,1-5,8 ; Zn 0-0,05 ; Bi 0,20-0,40 ; et Sn 0,20-0,50.

13. Composition selon l'une quelconque des revendications 5 à 12, ladite composition d'alliage d'aluminium présentant un rapport pondéral de Bi/Sn dans la plage allant de 1,32/1 à 0,8/1.

14. Composition selon l'une quelconque des revendications 5 à 13, dans laquelle lesdites impuretés accessoires sont présentes selon une quantité totale inférieure à 0,5% en poids.
